

## UNITED STATES PATENT OFFICE

2,110,792

PROCESS FOR ELECTRODEPOSITION OF  
SILVER AND PRODUCTS OBTAINED  
THEREFROMBirger Egeberg and Nathan Promisel, Meriden,  
Conn., assignors to International Silver Com-  
pany, Meriden, Conn., a corporation of New  
JerseyNo Drawing. Application March 23, 1936,  
Serial No. 70,396

10 Claims. (Cl. 204—16)

This invention relates to electrodeposits of silver and similar metals, including silver alloys, and to a process of electrodeposition thereof.

In the present accepted commercial practice of electroplating silver coatings, the standard bath is composed of silver cyanide, an excess of alkali cyanide over that required to dissolve the silver cyanide, alkali carbonate and water. Through this solution an electric current of suitable characteristics is passed, the current passing into the solution through silver anodes of high purity, through the solution depositing silver on the articles to be plated which constitute the cathodes, and then out of the bath through the cathodes. Under proper conditions of current, temperature, agitation and maintenance of a proper concentration of the electrolyte, a crystalline, non-lustrous matte white deposit of silver may be secured at the cathode. Buffing or burnishing, sometimes both, of such a deposit is, therefore, necessary to secure a bright surface. This buffing and burnishing is costly and wasteful and accordingly highly undesirable. It is, therefore, common practice to add to the above plating bath a brightener which will give the deposit, as it is made in the bath, a slightly lustrous appearance. For producing such a deposit, carbon-disulphide has been proposed and used commercially for nearly 100 years. A number of other brighteners have been also proposed such as gums, sugars, sodium thiosulphate, tellurium and selenium compounds and others. The only one in extensive commercial use, however, is carbon-disulphide and the other proposed brighteners have never come into extensive commercial use.

Carbon-disulphide although known and used for nearly a century has certain well-recognized disadvantages which may be briefly summarized as follows: Even under the best conditions the deposit is not satisfactory and frequently lacks any appreciable luster. It is, moreover, usually not uniform over the entire plated surface unless extreme precautions are taken. The deposit is sensitive to plating conditions in that the quantity of carbon-disulphide present, the current density, temperature, agitation and solution composition must all be adjusted and maintained within closely balanced limits. The carbon-disulphide limits are far narrower than required by the other components of the solution, namely,

the silver cyanide, alkali cyanide, carbonate and water. One difficulty in maintaining the proper quantity of carbon-disulphide present is that it is volatile at room temperature and this, in addition to its disappearance due to electrolysis, causes it to vanish rapidly from the solution making frequent additions necessary. Consequently, the precautions which have to be taken in dealing with this material are numerous. It is a fact that where many individual plating solutions including carbon-disulphide are used, even with the best of control, there are always certain solutions which perform unsatisfactorily and from which dull deposits are obtained, and even in solutions giving semi-lustrous deposits, there are always variations in appearance from vat to vat and even from section to section on the same article. In general, in employing this material, trial-and-error methods of plating have to be employed to secure the semi-lustrous deposits. Departure from conditions so determined may result in deposits the luster of which is actually inferior to those obtained from solutions containing no carbon-disulphide whatsoever. In addition, we have found with carbon-disulphide that only a relatively thin plating of semi-lustrous character can be obtained, in that, with increasing thickness of the deposit, the deposit changes from the semi-lustrous appearance to, eventually, a dull white appearance.

The principal object of the present invention accordingly is to provide a deposit or coating of silver that has as deposited an inherent, smooth, uniform, highly lustrous character even for the thickest commercial coatings. Another object of the invention is to provide a process for the production of such a deposit or coating which will do away with at least some of the objections to carbon-disulphide and other brighteners heretofore employed.

In accordance with our invention we have found that highly lustrous deposits or platings of silver may be produced under proper conditions of ingredient proportions and other characteristics of the solution and current employed, by electrolyzing a cyanide silver bath containing silver cyanide, alkali cyanide, and alkali carbonate in the presence of a brightener comprising any of several groups of chemical compounds, including derivatives of thio-carbaric acids, particularly

thio-carbamates, thio-ureas, thio-cyanates, urea or alkali metal cyanates, these substances, particularly the thio-cyanates, being such as not to produce ammonia since we find that the production of ammonia in our electrolytic baths interferes with the proper luster.

Certain of the compounds which constitute brighteners in accordance with the invention may be represented by the chemical formula

10



15. where X is  $\text{NH}_2$  or substituted  $\text{NH}_2$  in which one or both hydrogen atoms are replaced by the substituent radicals methyl, ethyl, acetyl or  $\text{NH}_2$ , and where Y is  $\text{NH}_2$ ,  $\text{SNH}_2\text{R}$ ,  $\text{SNH}_2(\text{R})_2$  or  $\text{SM}$  in which R is the methyl or ethyl radical, and 20 M an alkali metal.

20. The proportions of the brightener may vary from minute amounts for example 0.01 g/l to large quantities for example 100 g/l, depending upon the particular substance and the attendant conditions. By proper adjustment of the plating conditions a silver deposit is secured superior in luster to any such deposits or coatings heretofore produced. The deposits and plating bath also have to a much less extent the disadvantages 25 enumerated above for carbon-disulphide and in some cases these disadvantages are completely eliminated.

30. The following are preferred examples of baths and methods for carrying out the invention as we now prefer to practice it. It is understood that the invention is not to be considered as limited to these examples except as indicated in the appended claims.

#### Example 1

40

An electrolytic bath employing thio-urea

45



as a brightener is as follows:

|                         |       |    |
|-------------------------|-------|----|
| Silver cyanide          | grams | 25 |
| Potassium cyanide       | do    | 45 |
| 50. Potassium carbonate | do    | 20 |
| Thiourea                | do    | 45 |
| Water                   | liter | 1  |

55. At a temperature of 80° F. lustrous silver deposits may be obtained at a current density of 6 amperes per sq. ft. of cathode surface.

#### Example 2

60

Another example employing acetyl-thio-urea

65



is as follows:

The electrolytic bath contains:

|                     |       |    |
|---------------------|-------|----|
| Silver cyanide      | grams | 25 |
| Potassium cyanide   | do    | 45 |
| Potassium carbonate | do    | 20 |
| 70. Acetyl-thiourea | do    | 45 |
| Water               | liter | 1  |

75. At a temperature of 80° F. lustrous silver deposits may be obtained at a current density of 6 amperes per sq. ft. of cathode surface.

Another example employing mono-methyl-ammonium salt of mono-methyl-thiol-thiono-carbamic acid



is as follows:

The electrolytic bath contains:

|                                                                     |       |     |
|---------------------------------------------------------------------|-------|-----|
| Silver cyanide                                                      | grams | 25  |
| Potassium cyanide                                                   | do    | 50  |
| Potassium carbonate                                                 | do    | 50  |
| Mono-methyl ammonium salt of mono-methyl-thiol-thiono-carbamic acid | gram  | 0.5 |
| Water                                                               | liter | 1   |

At a temperature of 80° F. lustrous silver deposits may be obtained at a current density of 6 amperes per sq. ft. of cathode surface.

#### Example 4

An example employing potassium thiocyanate CNSK is as follows:

The electrolytic bath contains:

|                       |       |    |
|-----------------------|-------|----|
| Silver cyanide        | grams | 25 |
| Potassium cyanide     | do    | 45 |
| Potassium carbonate   | do    | 20 |
| Potassium thiocyanate | do    | 20 |
| Water                 | liter | 1  |

At a temperature of 80° F. lustrous silver deposits may be obtained at a current density of 6 amperes per sq. ft. of cathode surface.

#### Example 5

An example employing urea



is as follows:

The electrolytic bath contains:

|                     |       |    |
|---------------------|-------|----|
| Silver cyanide      | grams | 25 |
| Potassium cyanide   | do    | 45 |
| Potassium carbonate | do    | 20 |
| Urea                | do    | 45 |
| Water               | liter | 1  |

At a temperature of 80° F. lustrous silver deposits may be obtained at a current density of 6 amperes per sq. ft. of cathode surface.

Other substances which may be satisfactorily employed coming under the formula mentioned include—



Di-methyl-ammonium salt of di-methyl-thiol-thiono-carbamic acid



Mono-ethyl-ammonium salt of mono-ethyl-thiol-thiono-carbamic acid



Mono-methyl-ammonium salt or potassium salt of thiol-thiono-carbamic acid



75

The baths may be used immediately upon being prepared but we ordinarily prefer to allow them to age for two or three days before use.

5 The thio-cyanates, thio-carbamates, thio-ureas and urea described above may be prepared by known methods.

Certain of the above mentioned brighteners, for example, thiourea and urea, are substantially non-volatile, and the deposits resulting from 10 their use are substantially uniform and approach mirror brightness. Being of such high luster they require little or no polishing. With these substances the current density, temperature, agitation and solution composition may be varied 15 to the same extent as these factors vary in ordinary plating practice and it is not necessary, as in the case of carbon-disulphide, to adopt any extreme precautions to produce the deposit. These materials may be consumed during 20 electrolysis to some extent but in any case their replenishment is easy to take care of. No more frequent additions of these materials are necessary than required for the silver cyanide, alkali cyanide or carbonate of the bath. The range of 25 concentration of the materials as noted may be varied and accordingly the control of the concentration is not difficult.

We claim:

1. A process for the electrodeposition of silver 30 which comprises electrolyzing a silver cyanide bath containing a thio-urea as a brightener to form a bright deposit of silver therefrom.

2. A process for the electrodeposition of silver 35 which comprises electrolyzing a silver cyanide bath containing acetyl-thio-urea as a brightener to form a bright deposit of silver therefrom.

3. A process for the electrodeposition of silver which comprises electrolyzing a silver cyanide bath containing a mono-methyl-ammonium salt 40 of mono-methyl-thiol-thiono-carbamic acid as a brightener to form a bright deposit of silver therefrom.

4. A process for the electrodeposition of silver which comprises electrolyzing a silver cyanide 45 bath containing a thio-semi-carbazide as a brightener to form a bright deposit of silver therefrom.

5. As a new article of manufacture, a metal base having a surface electrodeposit of silver characterized by high and substantially uniform luster as deposited and requiring thereby a minimum of polishing, said deposit being obtained from a silver cyanide plating bath containing thiourea 50 as a brightener.

6. As a new article of manufacture, a metal base having a surface electrodeposit of silver characterized by high and substantially uniform luster as deposited and requiring thereby a minimum of polishing, said deposit being obtained 55 from a silver cyanide plating bath containing acetyl-thio-urea as a brightener.

7. As a new article of manufacture, a metal base having a surface electrodeposit of silver characterized by high and substantially uniform luster as deposited and requiring thereby a minimum of polishing, said deposit being obtained from a silver cyanide plating bath containing a mono-methyl-ammonium salt of mono-methyl-thiol-thiono-carbamic acid as a brightener.

8. A process for the electrodeposition of silver 10 which comprises: electrolyzing a silver cyanide plating bath containing a brightener having the chemical formula



15

where X is a member of the group consisting of NH<sub>2</sub> and substituted NH<sub>2</sub> in which the substituents for hydrogen are methyl, ethyl, acetyl or NH<sub>2</sub>, and where Y is a member of the group consisting of NH<sub>2</sub>, SNH<sub>3</sub>R, SNH<sub>2</sub>(R)<sub>2</sub> and SM in which R is methyl or ethyl and M an alkali metal, said substituting groups being such as not to make the resulting compound insoluble in 20 the cyanide plating bath and not forming a substance substantially alkaline in water or producing ammonia during the process of electrolysis.

9. As a new article of manufacture a metal base having a surface electrodeposit of silver 30 characterized by high and substantially uniform luster as deposited and requiring thereby a minimum of polishing, said deposit being obtained from a silver cyanide plating bath containing a brightener having the chemical formula 35



40

where X is a member of the group consisting of NH<sub>2</sub> and substituted NH<sub>2</sub> in which the substituents for hydrogen are methyl, ethyl, acetyl or NH<sub>2</sub>, and where Y is a member of the group consisting of NH<sub>2</sub>, SNH<sub>3</sub>R, SNH<sub>2</sub>(R)<sub>2</sub> and SM in which R is methyl or ethyl, and M an alkali metal, said substituting groups being such as not to make the resulting compound insoluble in 45 the cyanide plating bath and not forming a substance substantially alkaline in water or producing ammonia during the process of electrolysis.

10. As a new article of manufacture, a metal base having a surface electrodeposit of silver characterized by high and substantially uniform luster as deposited and requiring thereby a minimum of polishing, said deposit being obtained from a silver cyanide plating bath containing 55 thio-semi-carbazide as a brightener.

BIRGER EGEBERG.  
NATHAN PROMISEL.

60